

April 1, 1958

W. T. JACKSON

2,828,752

FIBROUS TOBACCO SMOKE FILTERS

Filed Aug. 16, 1954

4 Sheets-Sheet 1

**Fig. 1**



**Fig. 2**  
PRIOR ART



**Fig. 3**



**Fig. 7**

Wallace T. Jackson  
INVENTOR.  
Daniel I. Mayne,  
BY *John B. Hill Jr.*  
ATTORNEYS

April 1, 1958

W. T. JACKSON

2,828,752

FIBROUS TOBACCO SMOKE FILTERS

Filed Aug. 16, 1954

4 Sheets-Sheet 2



Wallace T. Jackson

INVENTOR.

BY Daniel L. Mayne,  
MURRAY J.

ATTORNEYS

April 1, 1958

W. T. JACKSON

**2,828,752**

## FIBROUS TOBACCO SMOKE FILTERS

Filed Aug. 16, 1954

4 Sheets-Sheet 3



Fig. 6

Wallace T. Jackson

*INVENTOR.*

INVENTOR.

Daniel L. Mayne  
BY John B. Hill Jr.

ATTORNEYS

April 1, 1958

W. T. JACKSON

2,828,752

FIBROUS TOBACCO SMOKE FILTERS

Filed Aug. 16, 1954

4 Sheets-Sheet 4

**SECTION OF SPINNERETTE  
SHOWING ONE ORIFICE**

**Fig. 8**



**Fig. 9**



**Wallace T. Jackson**

INVENTOR.

BY *Daniel J. Mayne*  
*John R. Jackson*

ATTORNEYS

2,828,752

## FIBROUS TOBACCO SMOKE FILTERS

Wallace T. Jackson, Kingsport, Tenn., assignor to Eastman Kodak Company, Rochester, N. Y., a corporation of New Jersey

Application August 16, 1954, Serial No. 449,872

11 Claims. (Cl. 131—208)

The present invention relates to tobacco smoke filtering material and elements thereof suitable for use in cigarettes, pipes, cigarette holders, and cigar holders. More particularly, the invention is concerned with a novel fibrous filtering material comprising an improvement in fibrous filters of the general type disclosed in pending U. S. patent applications of Crawford and Stevens, Serial Nos. 324,342, filed December 5, 1952, now Patent 2,794,239 of June 4, 1957, and 374,168, filed August 14, 1953, now Patent 2,794,480 of June 4, 1957, to each of which reference is made.

In the aforementioned applications, newly discovered advantages of a certain type of fibrous tobacco smoke filter are discussed. According to Crawford and Stevens, a filter is prepared from a continuous strand of filamentary material and comprises a structurally unitary rodlike mass of fibers and a wrapper encircling the mass, the fibers as a whole being in substantial alignment longitudinally of the mass but substantially each of the individual fibers having a plurality of short portions thereof crimped into diverging and converging relationship to the main fiber axis, a plurality of the fibers having physical bonds to contiguous fibers at random points of contact. Very good results have been obtained in the use of such filters for the removal of nicotine and tars from tobacco smoke, especially in view of the fact that the filters supply other requirements equally as necessary to the success of a tobacco smoke filter. A particularly advantageous embodiment of the Crawford and Stevens filter is that in which the filter is prepared from a synthetically spun, crimped, continuous filament tow, e. g. cellulose acetate. In this form, the rodlike mass therefore comprises a segment of the tow in which the fibers are coextensive with the mass. In its preferred form, the fibers of this filter have surface solvation bonds comprising coalesced portions of contacting fibers.

Filtering elements of the general type described above are prepared by the "cigaretting," i. e. by shaping and wrapping with paper a tow which previously has been subjected to a special preliminary conditioning treatment. The special treatment or preliminary conditioning of the tow was found to provide an advantageous character to the material thus treated whereby properties requisite to (a) good "cigaretting," (b) cigarette assembling (i. e. joining of the filter elements to wrapped bodies of tobacco), and (c) filtering are vastly enhanced. Thus, the preliminary conditioning method results in a tobacco smoke filtering element with quite a distinct character as respects compactness, size, density, smoke channeling, cross-sectional fiber distribution, air pressure drop, resiliency, body, feel, rigidity, fiber loss, porosity, integrity and the like. These properties are provided in such quantity and relationship that the material not only only is pleasing as a cigarette component but is susceptible of handling with processing apparatus normally used for cigarette manufacture and packaging. Also provided is the equally important requirement that in any given op-

eration the filamentary filter material produced exhibits its various characteristics uniformly and within close tolerance. The method is adapted for the continuous high speed conversion of crimped continuous filament tow to a smoke filtering material.

5 In its entirety, the method of Crawford and Stevens consists of the steps of (a) preliminary tow conditioning, (b) "cigaretting" of the thus conditioned tow with the formation of cured, paper wrapped fiber masses, and 10 (c) assembling of the complete cigarettes by joining the paper wrapped fiber masses to the paper wrapped tobacco rods comprising the main portion of the cigarettes.

The preliminary step of tow conditioning consists essentially of two principal operations: (1) filament separation, and (2) creation of an adhesive attitude among the separated filaments. A third and more or less incidental step involves the orderly collection of the filaments of the treated tow under controlled conditions of tension and uniform presentation of the collected tow 20 to a cigaretteting means, e. g. a garniture.

Perhaps the most critical phase of the entire conditioning process is the step of filament separation which has been found to provide two requisite qualities to the tow. First, filament separation amounts to an opening 25 of the tow in the respect that small compact bundles of filaments within the tow are broken up to give a more uniform cross-sectional distribution of filaments throughout the entire tow. Uniformity manifests itself in the final product primarily through reduction in the normal 30 tendency of the filtering material to cause channeling of the smoke through areas in which the fiber density, i. e. distribution of fibers is less than in other areas. Uniformity also manifests itself in an improved compactness, rigidity and resiliency of the product. Another characteristic imparted to the tow in filament separation is the 35 susceptibility, i. e., exposure of all or a large percentage of the individual filaments to treating materials in the subsequent conditioning step, i. e. in the creation of an adhesive attitude among the filaments. In other words, 40 the step of filament separation results in the individual filaments being more vulnerable to a fluid treatment as well as in their having a condition wherein the filaments assume a more uniform and dechannelized (debundled) transverse distribution of fibers. Exposure and susceptibility 45 are manifested in the final product through an improved retention of uniformity, and through improved rigidity, resiliency and integrity.

It has been taught by Crawford and Stevens that filament separation is best accomplished through at least two 50 distinct operations on the tow, each of which promotes both uniformity of distribution and exposure, but the first achieving primarily distribution and the second achieving primarily exposure. Thus, it has been indicated to be advantageous to conduct filament separation 55 by means of the successive steps termed tow opening and tow banding, respectively.

By "banding" is meant widening at the expense of thickness. Thus, a "banded" tow is one which has been converted to a web-like, i. e. ribbon-like conformation 60 being, for instance, five to sixteen (usually about eight to fourteen) times its original width and having little thickness so that all or at least a substantial majority of the individual filaments are directly exposed and vulnerable to a spray from one or both sides of the banded web. In other words, "banding" may be described as an operation for greatly increasing the dimension of the tow in a first plane while maintaining a substantially uniform distribution of fibers in that plane and greatly 65 reducing the dimension of the tow in a second plane perpendicular thereto. Banding is accomplished by means 70 tending to move the filaments apart by movement more

or less confined to a single plane and therefore banding assists in the dechannelizing and debundling of the tow. At the same time, a prior debundling of the tow appears to be necessary to the success of the banding operation.

Debundling is largely accomplished by the operation of tow opening preceding the banding step. Opening is nicely procured by the use of tensional forces which take advantage of the inherent springiness of the tow to restrict it to an extent from which its reaction, upon release of tension, is to open or expand. Thus while opening also facilitates banding, it primarily promotes uniformity of filament distribution in the tow. Opening thus is important in providing a debundled and dechannelized structure in the final product. In accordance with the terminology used herein, a "dechannelized" tow is one in which there has been eliminated or substantially reduced any tendency for smaller groups of adjacent filaments to become associated as distinct compacted smaller bundles within the larger mass or bundle of filaments. Such a tendency of course inherently includes a tendency toward formation of channels. It is necessary to remove and break up such grouping in order that there be no small fiber bundles present in the final product.

Therefore, a preferred method for the conversion of cellulose acetate tow into tobacco smoke filter elements comprises the successive steps of (1) conducting filament separation by (a) opening, i. e. enlarging the diameter of a crimped tow supplied continuously, and (b) banding the thus opened tow to form a ribbonlike web of relatively large width and small thickness, (2) creating an adhesive attitude among the filaments of the banded tow by subjecting the latter to a spray of liquid plasticizer, which has a solvent action on the filaments, (3) collecting the treated tow and presenting it to cigaretteting means under uniform conditions adapted to retain within the tow characteristics imparted to it in the first step, (4) cigaretteting the thus conditioned tow by condensing, shaping, wrapping, sealing and severing it into desired lengths, and (5) stiffening the elements severed from the continuous length of material so produced by a curing treatment, i. e. aging, heating, or both. The stiffened elements in suitable length then may be joined each to the tobacco body of a cigarette as a filter tip, or they may be employed each in a suitable length as a filter unit for a cigarette or cigar holder or pipe.

It has been appreciated for some time that possibly the most critical step in the continuous conversion of running lengths of crimped continuous filament tow into cigarette filters by the general method as described above perhaps is the step of tow opening, which takes place as a part of the filament separation phase. The ease of subsequent processing of the tow in standard apparatus as well as the character of the final product appears to be very extensively influenced by the manner of and success with which the tow opening step is conducted. Tow opening normally is accomplished continuously by means of a device which consists of two pairs of cooperating tensioning rolls spaced along and forming a path for movement of the tow successively through the bites of the roll pairs. The downstream pair is positively driven to grip and pull the tow against a restraining force applied by the upstream pair of rolls which is composed of rolls retarded either by frictional braking or by being positively driven at a slower speed than the positively driven tensioning rolls. The tension exerted on the tow by the downstream rolls in overcoming the retarding effect of the retarded rolls, which tension normally may be of the order of about 20 to 50 pounds, serves to straighten out the crimp in the tow whereupon at the emergence of the tow from the nip of the tension rolls into a zone of relative relaxation, i. e., relatively little tension, the tow undergoes an expansion, i. e., enlargement of diameter and circumference and reduction of fiber density transversely, through the spring-like action of the fila-

ments in returning to their normal crimped condition, and causing a puffing up of the tow body. That is to say, a type of explosive expansion occurs within the tow to provide bundle breaking, i. e., disintegration of any individual compact bundles of filaments which may exist within the larger bundle forming the tow.

In other words, the tensioning apparatus subjects the tow to sufficient tension to produce a restriction of substantially each strand which straightens the strand by "pulling out" the crimps and results, upon emergence of the strand from the nip of the positively driven rolls into a zone of relative relaxation, in a more uniform distribution of filaments within the strand as a result of inherent and elastic forces within the filaments of the strand. These forces are exerted transversely by each filament in reassuming its crimped configuration and thus are exerted transversely of the strand and are more intense where filament density, i. e., the concentration of filaments is greatest. Therefore, the lateral forces cause transverse displacement of filaments from zones of high filament density. Thus action herein termed "tow opening" or "bundle breaking" obviously is dependent upon the use of both (a) satisfactorily crimped and springy tow and (b) zones of definite tension differential.

As suggested above, it is known that the more complete the blooming action produced by the tensioning step, the more easily the tow is processed in the equipment of the tobacco industry and the more perfect the character of the filter tips so manufactured. The present invention provides for improvement in the step of filament separation and a consequent improvement in the physical character of the final product thereby produced as regards adaptability for the cigaretteting and assembling and its utility as a tobacco smoke filtering element. While the use of countless types of fibers, both natural and synthetic, has been suggested, I am not aware that anyone has ever investigated the significance of shape characteristics of the fibers, e. g. the cross-sectional shape of the individual fibers. Indeed, there is nothing in the art to indicate that any given fiber section will have any particular influence on the utility of that fiber as a tobacco smoke filtering material. As a consequence, discussions of synthetically spun materials, so far as I am aware, have always been in terms of the normal or usual fiber sectional shapes as employed in the textile art. In other words, in the aforementioned Crawford and Stevens applications, synthetic fibers, e. g. cellulose acetate, were described as being preferably, for example, a "yarn-type" acetate containing about 38.8% to 39.2% acetyl, etc. This material normally would be spun from round holes of a size depending upon the desired filament denier, and would after solvent removal and solidification, have a somewhat irregular cross-section roughly in the shape of a clover leaf.

While such filaments react quite satisfactorily to the conditioning treatment, I now have found that a new dry spun cellulosic filament of novel cross-sectional shape gives an exaggerated reaction to the tow conditioning treatment of the method of Crawford and Stevens and thereby produces a product of very substantially enhanced character as regards processing ease in all of the subsequent steps (1) conditioning, (2) cigaretteting, and (3) assembling, and as regards uniformity and quality of the product filtering elements prepared thereby.

Accordingly, it is a primary object of the present invention to provide a new and improved fibrous tobacco smoke filter element. A second object of the invention is to prepare tobacco smoke filters from synthetically spun continuous filament tow composed of filaments having a Y-shaped cross-section. A still further object is to prepare fibrous filters of improved physical properties. Another object is to enhance the blooming, i. e. tow opening in the conditioning of a crimped continuous filament tow for use in preparation of tobacco smoke filters. Another object is the preparation of a filter element com-

posed of fibers having a Y-shaped cross-section. A still further object is to provide a filter having increased bulk, resiliency and body. Another object is to provide a filter element where the superior bulk of the component Y-shaped filaments provides a more tightly packed rod without increasing its pressure drop. Another object is the preparation of a fibrous filter having aligned fibers of a more uniform cross-sectional fiber distribution. Other objects will be apparent in the following specification and claims.

The present invention resides in a tobacco smoke filtering element comprising an elongated structurally unitary rodlike mass of crimped synthetically dry-spun fibers and an annular wrapper encircling the mass, each fiber of the mass being substantially coextensive therewith, the fibers as a whole being in substantial alignment longitudinally of the mass but substantially each of the individual fibers having non-oriented short portions thereof disposed randomly in diverging and converging relationship to the main fiber axis, a plurality of the fibers having surface solvation bonds to contiguous fibers at random points of contact, a substantial portion of the fibers having a substantially uniform Y-shaped cross-section, the Y-section having legs of substantially equal length and of substantially equal shape, and the angles between adjacent legs of the Y preferably being substantially equal. Most advantageously the fibers of the invention are prepared from single or mixed organic acid esters of cellulose derived from acids containing 2 to 4 carbon atoms, the filaments having a size of 1.5 to 43 denier. Most advantageously the filaments are of cellulose acetate.

The invention is illustrated in the accompanying drawings in which

Figure 1 is a reproduction of an actual photomicrograph showing the cross section of several Y-shaped filaments of which the tobacco smoke filters of the present invention are made,

Figure 2 is a reproduction of an actual photomicrograph showing in cross section several clover-leaf filaments made by the customary prior art method,

Figure 3 is an enlarged longitudinal section through a portion of a tipped cigarette assembled with a filter of the invention,

Figure 4 is a diagrammatic representation of the steps of the method for preparing a filter of the invention,

Figure 5 is a top plan view, partially cut away, of a preferred form of apparatus for conducting the method of the invention,

Figure 6 is a side elevation, partially cut away, of the apparatus of Figure 5,

Figure 7 is a view of the face of a spinnerette showing a plurality of filament forming orifices of equilateral triangular shape for dry-spinning Y-shaped filaments suitable for the new tobacco smoke filtering element.

Figure 8 is a greatly enlarged representation of a spinning solution coming out of the triangular orifices of a spinnerette such as represented in Fig. 7 and forming into Y-shaped cross-section filaments, and

Figure 9 is a schematic elevational view, partly in section, showing a spinnerette which has equilateral triangular filament forming orifices positioned in a suitable dry spinning cabinet which is equipped with suitable auxiliary apparatus.

The filamentary material used for the filters of the present invention and methods for its preparation are disclosed and claimed in Raynolds, Abernathy and Smith U. S. patent application Serial No. 400,564, filed December 28, 1953. The material may be prepared by forcing a suitable spinning solution through a spinnerette having a plurality of equilateral triangular shaped filament forming orifices therein and evaporating the solvent by drying the resulting filaments in a spinning cabinet under carefully controlled conditions of temperature while subjecting the filaments to predetermined drafting. The

temperature of the solution and its rate of extrusion are so controlled as to secure optimum results.

Under the optimum conditions of solution temperature and composition, and of extrusion, drying and drafting, the wet filaments as they leave the equilateral triangular orifices temporarily assume a triangular cross-sectional shape. However, by careful control of the extrusion rate, the drafting rate and drying temperatures, there is produced a change in the filament cross-section from a triangular to a Y-shaped cross-section. Under preferred ranges of operation the "legs" of the Y-shaped cross-section filament will be substantially equal in length and of substantially uniform shape. Also the angles between adjacent legs of the Y will be substantially equal. The Y-shaped cross-section is uniform along the length of the filament.

In general the spinnerette having the equilateral triangular orifices may be employed with any suitable spinning cabinet such as, for example, one of the forms illustrated in U. S. Patent 2,000,047 and 2,000,048.

The characteristics of the filaments and fibers used in the present invention may be due to the intermeshing of the legs of the Y of the individual filaments in the filament bundle in such manner that each is reinforced by the other and the filament bundle has a resultant stiffness greater than that possessed by the normal cross-section fiber of equivalent denier because of the increased surface area. Such an arrangement would appear to result in increased blooming action and uniformity of fiber distribution. It is noted that a circle taking in the three tips of the legs of the Y will be greater in diameter than one taking in the lobes of the well-known clover-leaf type of cross-section. This larger "circle" is, therefore, the effective area of the Y-shaped cross-section and may explain the increased utility of the Y-type of filament and fiber for tobacco smoke filters. However, it cannot be definitely stated on what basis the improved filters and improved tow opening are achieved.

Referring to Figure 9 there is shown schematically a side elevation view, partly in section, of a spinning cabinet 11 and its associated apparatus by which the novel Y-shaped synthetic filaments and fibers may be manufactured. Mounted at the top of the cabinet is a candle filter unit 12 to which is connected a spinnerette 13 which has a plurality of orifices 14 therein which are of the shape of equilateral triangles. The face of this novel type of spinnerette with the equilateral triangular orifices 14 therein is shown in the greatly enlarged view of Figure 7. The candle filter may be uniformly heated by means of heating coils, not shown, which are positioned so as to surround candle filter 12, and through which coils may be circulated any appropriate heat exchange medium such as water maintained at the desired temperature.

Spinning solution of composition described hereinafter is supplied from conduit 16 through valve 17 to pump 18 which forces the solution at the desired rate to the candle filter unit 12, thence to spinnerette 13 through the equilateral triangular orifices 14 from which it is extruded initially in the form of equilateral triangular filaments 25.

The filaments 25 pass downwardly in the cabinet 11 while progressively losing solvent by evaporation until, in a substantially solidified condition they leave the cabinet 11 and pass around godet roll 20, which is positioned below the lower end of the spinning cabinet 11. Godet roll 20 is driven at a uniform speed by means, not shown, to give the desired draft to the filaments 25. From godet roll 20 the filaments pass in the usual guide and are collected and assembled through other guides (not shown) with filaments from other spinning cabinets, moving at the same speed, to form a tow of a desirable number, e. g. 3000-30,000 continuous filaments. The tow is then sent through a crimping machine wherein a crimp of e. g. 2-16 crimps per inch is applied, and the tow is then formed into a package, e. g. a ball warp, for transport to

filter making machinery. The tow is lubricated, preferably adjacent the godet roll, with a non-toxic non-static reducing lubricant such as mineral oil.

To facilitate the evaporation of solvent from the filaments during their travel through the cabinet, heated air is supplied to the cabinet 11 by means of inlet conduits 23 and 24 positioned respectively adjacent the lower and upper ends thereof, the air passing through the cabinet and emerging through outlet conduit 26 positioned at a substantial distance below spinnerette 13, as illustrated.

The change of the cross-section of the filaments while in the cabinet from an initial triangular cross-sectional shape to the desired Y cross-sectional shape is illustrated in Figure 8. As shown at 25 the filaments have just been formed by the triangular orifices and are substantially of an equilateral triangular cross-section. Further on in the downward progress of the filaments under the controlled condition of drafting and drying they have changed to the desired Y cross-section filaments 25 which are depicted greatly magnified in Figure 8.

The general process for the preparation of dry spun Y-type filaments from cellulose acetate is described in the following example.

*Example 1.*

A spinning solution consisting of 26.5% cellulose acetate, 1.25% titanium dioxide, based on the weight of the cellulose acetate, 1.75% water and the remainder being the solvent, acetone was spun into Y-shaped cross-section filaments of 1800 denier per strand using the apparatus and its general operation as described above in connection with Figure 9. The spinnerette had 600 equilateral triangular orifices therein.

Thus, the method of Y filament formation from a cellulose organic acid ester, e. g. yarn-type cellulose acetate may be said to comprise the steps of extruding a cellulose organic acid ester filament forming solution through a spinnerette equipped with equilateral triangular extrusion orifices and into a dry spinning cabinet, drafting the thus formed triangular cross-section filaments at a draft ratio within the range of approximately 1.10 to 1.43 whereby the cross-section of the filaments is changed to said Y cross-section while drying the filaments at an average temperature within the range 40° C. to 90° C.

After the crimped tow of Y-shaped cross-section filaments has been prepared, packaged, and transported to a filter manufacturing facility, it is fed to a filter making apparatus for conversion into tobacco smoke filters through the successive steps of (1) conditioning and (2) cigaretteing. As stated above, it is preferable to employ a textile yarn-type acetate having an acetyl value of 38-41% (preferably 38.8-39.2%) in the form of a continuous filament tow having between 5,000 and 100,000 filaments (preferably 20,000) of about 1.5 to 16 (preferably about 5) denier per filament or a total denier within the range 60,000 to 250,000 (preferably about 100,000), all filaments having about 4 to 18 (preferably 9) crimps per inch and being conditioned with a "semi-lubricant." Modern textile lubricants furnish both lubricating and anti-static action. By a "semi-lubricant" is meant a lubricant which furnishes lubrication only, thereby producing a tow carrying a static charge to assist in filament separation and distribution. A preferred lubricant is a neutral, non-toxic material, most advantageously about 0.5% of pharmaceutical grade mineral oil by weight of the fiber.

In regular cigarette manufacture, shredded tobacco is metered from a hopper onto a moving paper ribbon carried by a flat tape. The tobacco and the paper then go through one or more dies thus forming the tobacco into a cylinder and lapping the paper over itself. Then glue is applied along the overlapping edge, the edge is smoothed down and the joint is heat-sealed, forming a continuous cigarette. A cutter knife cuts the tube into desired lengths. Thus my invention in the cigarette

step involves passing a properly conditioned tow of cellulose acetate filaments in a continuous manner through a cigarette manufacturing machine, i. e. the garniture of a cigarette manufacturing machine in which the tow is formed and shaped into a cylindrical section having the approximate diameter of a cigarette body, wrapped in paper, with the paper joint being sealed, and severed into the paper covered rods of appropriate length.

A highly useful method in accordance with the invention comprises as the step of creation of an adhesive attitude in the fibers the application of a spray of liquid adhesive or a liquid which will cause the filament surfaces to become adhesive. In the most advantageous embodiment of the invention in which a yarn type cellulose acetate continuous filament tow is employed, the step of creating an adhesive attitude is conducted in terms of a spray of a liquid plasticizer effective to produce a surface solvation in those portions of the acetate filament surface contacted by the plasticizer. The plasticizer partially dissolves or softens the fiber which it reaches and produces therein a sticky attitude sufficient to subsequently produce bonding between filaments having adjacent contacting areas affected by plasticizer. Thus, by the term "surface solvation" of the fibers as used herein is meant the creation, by the action of a solvent or plasticizer and/or heat, of an adhesive, tacky or readily bonding condition of the fibers by solution or incipient solution of surface portions of the filament material whereby there is produced a welding and adhesion between adjacent filaments contacting at such portions, and by "coalescence" I mean the situation caused by partial or incipient solvation of surface portions of the filaments and resulting in a condition within those portions under which the portions will flow into or unite with similar portions of dissolved or plastic material in contiguous filaments.

Basically, apparatus for carrying out the invention comprises the combination with a cigarette machine of means operated synchronously therewith for conditioning the tow, the conditioning means comprising a plurality of cooperating means positioned successively along and forming a path for the tow and including a filament separation means disposed to withdraw tow from a source of supply, means adjacent the separation means for applying a fluid medium to the separated tow, and means positioned between the fluid applying means and the cigarette machine for uniformly collecting the treated filaments of the tow under conditions of controlled tension and uniformly presenting the collected tow to the cigarette machine. More specifically, a highly useful conditioning means comprises a group of successively positioned cooperating apparatus members comprising a tow opening apparatus, a tow banding apparatus, a fluid treating apparatus, and a collecting and presenting apparatus.

The most advantageous assembly of apparatus which has been found to be suited for providing uniformity of product in a high speed tow conditioning and filter forming method (e. g., a method operated at 100 to 200 feet of tow per minute) is illustrated in Figs. 5 and 6 in which the tow is represented diagrammatically only. With reference to these figures, the apparatus comprises an assembly of cooperating means successively positioned along and forming a path for tow 49 supplied from a ball warp 11 mounted for free rotation. Smooth arc-like metal members 12 and 13 serve as stationary friction fingers to remove slack from tow withdrawn from the ball warp 11. Proper slack removal prior to the filament separation operation helps avoid false twist in the tow and facilitates the conduct of the separation step. For best results the tow should be delivered to the filament separating means under a fairly constant tension.

A filament separation means comprising a tow opening apparatus consisting of a tensioning device having a pair of driven rolls 14 and a pair of frictionally braked re-

tarred rolls 15 serves to pull the tow from the ball warp and subject it to a predetermined tension for the distance of the ratch, i. e. the distance between the nips of the roll pairs 14 and 15. The tensioning device is powered from a prime mover 16 through a speed reduction gear box 36, shaft 45, and a chain and sprocket arrangement to sprocket 39 which is free to turn on a shaft 46, the shaft 46 being normally free to remain stationary during rotation to the sprocket 39. Integral with the sprocket 39 is a clutch plate 47. A cooperating clutch plate 48 is keyed to the shaft 46 and its position on the shaft 45 controlled by a bell crank 37 adapted for manual operation. Movement of the bell crank handle in the direction indicated by the arrow in Fig. 5 results in engagement of the clutch plates 47 and 48 and thereby provides actuation of the shaft 46 keyed to clutch plate 48. Rotating with the shaft 46 is a sprocket 50 through which power is transmitted to the roll tensioning device by means of chain drives 51 and 52, a variable speed transmission 17, and a chain and sprocket drive between the latter and the pair of rolls 14. The upper roll of the pair 14 is powered to rotate in a direction counter to the lower roll of the pair 14 in the direction as indicated by the arrows in Fig. 6. The action of these rolls 14 through the nip provided therebetween serves to pull tow from and through the braked rolls of the pair 15. The rolls of the pairs 14 and 15 have elastic cushioning surfaces to provide sufficient traction on the tow. The rolls of the retarded pair 15 are spaced sufficiently close to deform the cushion surface and introduce resistance through the friction of deforming. This provides a braking action by means of which a predetermined amount of tension, for example, of the order of 20 to 250 pounds, is imparted to the tow in the ratch between the two pairs of rolls. During the application of tension the crimp in the tow is straightened out and upon emergence of the tow from the nip of the drive rolls 14 into a relatively relaxed state, the tow undergoes an expansion, i. e. enlargement of diameter and circumference and reduction of fiber density transversely, through the puffing action or spring-like action of the filaments in returning to their normal crimped condition.

As mentioned above, the action of the tensioning apparatus is dependent upon the existence of an adjacent zone to which the tow passes after tensioning and in which the tow is subject to relatively little tension. This is brought about by the use of a feed roll assembly indicated generally by the arrow at 18 and comprising a pair of drive rolls which are used to move the tow away from the tension zone, into and through banding apparatus, into and through a spray chamber and to collect from the spray chamber the treated filaments of the tow uniformly under controlled tension conditions. The feed roll assembly also serves to present the thus collected tow to the cigaretteting means. The feed rolls are controlled synchronously with the cigaretteting machine and the tensioning device in such a manner that they withdraw tow from the latter and feed to the former as required, under a tension of very small order, i. e. sufficiently merely to pass the tow through the banding and spraying means without allowing the accumulation of excessive slack. Thus, it may be said that movement of the tow between the tensioning device and the collecting device is a matter of little more than removal of the slack existing in the tow adjacent the tensioning means.

From the point of emergence from drive rolls 14 of the tow opening apparatus the tow is pulled under the relatively little tension afforded by means of the action of the feed roll assembly through the second unit of the filament separation means which is an adjacent banding apparatus in the form of air jet banding devices 19 and 19a. The banding apparatus is spaced from the opening device a suitable distance, preferably at least about four times the banded width of the tow, to provide for gradual widening of the tow. The banding devices 19 and 19a

may each comprise a pair of parallel, spaced, oppositely disposed flat plates providing a slot-like aperture for passage of tow therethrough, at least one plate of the pair being provided with openings for forming jets of air or other gas under pressure. In the apparatus illustrated, air is fed under pressure through lines as indicated into plenum chambers below the tow path. Apertured plates form upper walls of these chambers and permit air jets to be directed against the tow. The slot provided between the upper and lower plates is shallow and sufficiently wide to accommodate the tow in the widest condition desired. The outer boundaries of the slot are formed by imperforate side walls. The banding jet devices may be of the type disclosed and claimed in my U. S. patent application Serial No. 356,983, filed May 25, 1953 now Patent 2,737,688 of March 13, 1956. The action of the jets of the banding jet device is to strike the tow perpendicularly to its path of movement and force the filaments apart, thereby forming a ribbon-like web having approximately eight to sixteen times the original tow width with a minimum of thickness. In this condition the filaments of the tow are accessible to fluids which are applied by the next member of the conditioning assembly. In using the two successive banding devices 19 and 19a, the first is smaller than the second and allows for gradual and more efficient banding by stagewise action.

From the banding apparatus 19 the tow emerges into a spray chamber 20 which is illustrated as having a slideable glass window and an exhaust hood and flue. In the spray chamber, a fluid bonding medium is applied by means of oppositely disposed spray guns 21 and 22 to produce an adhesive attitude in the filaments. Most advantageously the spray is a liquid plasticizer having a solvent action which will produce a tackiness in the filaments through surface solvation thereof at points of contact therewith of the liquid particles of the spray.

The plasticizer is fed to the spray guns 21 and 22 from a supply tank (not shown) and lines leading through solenoid valves 38 and 60. These valves are opened to admit plasticizer to the guns by energization of a circuit controlled by a suitable switch such as a spring-biased single throw switch or micro switch 61. The switch remains open when the apparatus is inoperative. When the clutch plates 47 and 48 are brought into engagement by movement of the bell crank handle in the direction indicated, the arm of the lever moving the clutch plate 48 contacts the switch and moves it into a position closing the circuit and thereby supplying plasticizer to the spray guns. This cooperation of elements prevents the application of an excessive amount of plasticizer to the banded tow if operation of the machine must be temporarily halted. The supply of pressure air to the spray guns may be controlled in a similar way but this is not necessary.

The plasticizer forms minute droplets at random points along the surface of substantially each of the filaments of the tow in sufficient quantity so that substantially each of the filaments will have a plurality of points of surface solvation along any length corresponding to the length of the smoke filtering unit which is to be the ultimate product.

Most advantageously, a plasticizing agent such as dimethoxyethyl phthalate or methyl phthalyl ethyl glycolate (carbethoxymethyl methyl phthalate) is employed. Other suitable nontoxic plasticizers which have nontoxic decomposition products and do not adversely affect the taste of tobacco smoke filtered through elements of the invention are dibutyl phthalate, tripropionin and acetyl triethyl citrate. The plasticizing agent preferably is sprayed on until the fibers contain 4 to 30% (preferably about 6-15%) by weight of plasticizer. If desired, the temperature at which the fluid treatment takes place may be controlled.

In the course of its continuous movement the tow, wet 75 with plasticizer, passes out of the spray cabinet 20 through

a slot in the side wall thereof and is received by a tow fluffing means as described in the Crawford and Stevens applications or preferably by a feed roll assembly such as 18.

The feed roll assembly 18 comprises an upper roll 70 around which the tow passes and a lower roll 71 which provides in cooperation with the upper roll 70 a nip for positive feeding of the tow through the feed roll assembly. The lower roll is powered by a sprocket arrangement including chain 72 transmitting power from a variable speed transmission unit 73 which in turn receives its power from the prime mover 16 through the sprocket arrangement including chain 51. The upper roll 70 may be powered to turn with the lower roll 71 or may receive its drive merely by frictional engagement with the tow and/or lower roll 71. From the lower roll 71 the treated tow 26 passes up and into the horn 25 of the garniture.

Tow is discharged from the feed roll assembly and presented to a capping means such as a garniture, i. e. cigarette-making machine into which it is drawn by the gripping and pulling action of the machine. The horn or die 25 of the garniture condenses and shapes the conditioned tow and discharges it onto a moving strip or ribbon of cigarette paper carried on an endless belt conveyor.

In the operation of a suitable type of garniture, as is well known in the art, the material being received, in this case the conditioned tow 26, enters the condensing horn (e. g. 25) and is continuously discharged therefrom onto paper web fed from a roll at the same linear speed as the material being received. The paper is lapped around the material, i. e. the rod of acetate filaments, in a shaping member and a standing edge of paper has adhesive continuously applied to it by a rotating disc. The standing paper edge is smoothed down over the adjoining edge by a stationary member and is heat-sealed into a permanent adhesive bond by a heated member. A rotating knife severs the paper-covered rod into appropriate lengths.

The garniture or capping machine may be powered by the prime mover 16 through the clutch plates 47 and 48 in a manner as explained above in connection with the tensioning device. A continuous conveyor belt 62 (Figs. 2 and 3) is driven through the action of pulley 63 which is keyed to the shaft 46. Other operating parts of the garniture may be synchronously driven by any convenient arrangement of shafts (not shown) geared to the shaft 46. In any event, the driving arrangement preferably is such that movement of tow through the entire apparatus and application of plasticizer are both controlled by means of the operation of the bell crank lever 37. Movement of tow and spray application thus are started and stopped in unison.

If desired, the paper covered rod formed by the capping operation may be stiffened by a heat curing treatment accomplished during passage of the rod through a heated member prior to severance. The same result may be obtained by subjecting the severed rods to heat treatment such as for instant storage in a chamber heated to 200° F. for a period of about two hours.

It is satisfactory to subject the finally wrapped rods of cellulose acetate filaments to a temperature of 160° F. for four hours where solvation has been accomplished with a plasticizer such as carbethoxymethyl methyl phthalate, although the treating time may be varied from 1/2 to 24 hours depending on the temperature and the particular plasticizing agent employed. Any temperature within the range of 125° F. to 300° F. may be found satisfactory. It sometimes may be satisfactory to forego a final heat treatment and merely to allow the paper-wrapped rod to age at room temperature for a period of for instance, 24 hours to allow the plasticizer to penetrate and the bonding to become thorough and complete.

After the paper-covered rod has been severed into elements of appropriate length and suitably cured, the elements may be employed as the final product for use in

5  
10  
15  
20  
25  
30  
35  
40  
45  
50

cigarettes, pipes, and cigarette and cigar holders. If the filter material is to be used as a tip for cigarettes, known procedures for manufacturing filter tip cigarettes may be used. That is to say, elements of appropriate length may be fed to a joiner or other assembling machine which serves to position the filter elements adjacent to tobacco bodies, join them and cut the joined pieces at the proper points.

The product produced in accordance with the present invention is an article of manufacture or smoking device containing the same, the article comprising a rod, normally cylindrical in form and customarily substantially the size of a cigarette in circumference and diameter, the rod being a compact, rigid, structurally unitary debundled mass of crimped cellulose acetate filaments of Y-shaped cross section, and a wrapper encircling the mass, each filament of the mass being substantially coextensive therewith, the filaments as a whole being in substantial alignment longitudinally of the mass but substantially each of the individual filaments having non-oriented short portions thereof disposed randomly in diverging and converging relationship to the main filament axis, substantially all of the filaments of the mass being positively bonded to contiguous filaments within said structurally unitary rod at random points of contact of the filaments, the filaments of the mass being uniformly distributed throughout the transverse section of the mass thereby providing a dechannelized condition within the mass.

Thus a "rod" in accordance with the terminology in this specification comprises a fiber mass, regardless of length or diameter, which results from conditioning and capping a tow according to the invention and which is structurally unitary or substantially so, and capable independently of substantially retaining its size and shape. The rods of the invention, though endowed with compactness and rigidity, are resilient and to a certain extent flexible. The rigidity of the rod may be emphasized almost to the point of inflexibility by means of a final curing treatment of proper intensity.

The condition and disposition of the filaments within the product is one in which the filaments, though members of the same strand and coextensive, are in less than exact longitudinal alignment due to the filament separation operation, and particularly to the individual short diverging and converging portions of the filaments comprising the crimps. Furthermore, the porosity and perviousness of the rod-like mass is preferably such that in passing longitudinally through the mass any given amount of tobacco smoke is split into numerous small streams and each stream guided through small channels formed by the surfaces of each group of adjacent filaments, channel size being such that good contact is thereby afforded between the filament surfaces and all portions of the smoke.

While the apparatus disclosed in the foregoing paragraphs has been found to be most advantageous for reproduction of uniformity in products produced according to the described method it should be mentioned that some alternatives for individual elements are possible within the scope of invention. For instance in the step of filament separation, tow opening may be accomplished by use in cooperation with a pair of drive rolls of a trap box having a weighted tongue to produce a braking action. The trap box would be a substitute for the pair of braked idler rolls 15. In other words, an opening device instead of two pairs of tension rolls might comprise a pair of driven rolls and a retarding device such as a tongued-trap box. Tow opening may be considerably enhanced through use, in combination with the two pairs of tension rolls, of a reciprocating striker mechanism operating in a plane adjacent and normal to the tow path in the tension zone between the two pairs of tension rolls. Such a mechanism is disclosed and claimed in copending Smith, U. S. patent application Serial No. 416,010, filed March 15, 1954, now Patent No. 2,790,208.

of April 30, 1957. By employing about 3500 strokes per minute to deflect the tow path about 2 to 3 inches per stroke, the method results in the periodic application to the already tensioned tow of a suddenly applied and suddenly released additional increment of tension sufficient to impart approximately an additional 8% stretch to the tow. This procedure improves and multiplies the opening effect to a substantial degree. It is less necessary, however, in preparation of the filter elements of the present invention than in preparation of elements from fibers of ordinary cross section.

Banding might be accomplished successfully through the use of an expander bar as known in the art or as suitably modified. Thus one might employ a banding device comprising a surface presenting a portion of a cylinder and provided with two diverging sets of tow contacting ribs at an angle to each other of, e. g., 60°. With such a device it is contemplated that tow passing over the bar and in frictional engagement therewith will be banded in a manner similar to that occurring in the banding jet in that filaments would be transversely moved apart from each other, particularly in regions of high filament density to produce a tow structure having a greatly increased uniformity of cross-sectional fiber distribution.

I claim:

1. A tobacco smoke filtering element comprising a structurally unitary, elongated, rod-like mass of cellulose acetate filaments and a wrapper encircling the mass, said mass comprising a segment of a crimped tow of continuous filaments, the filaments generally being in substantial alignment longitudinally of the mass but substantially every individual filament having non-oriented short portions thereof disposed randomly in diverging and converging relationship to the main filament axis, substantially every filament having surface solvation bonds provided by coalesced portions of contacting fibers, said portions containing a plasticizer having a softening action on the filaments, at least a substantial portion of the filaments having a substantially uniform Y-shaped cross section and the filaments of the mass being uniformly distributed throughout the transverse section of the mass thereby providing a dechannelized condition in the element.

2. A tobacco smoke filtering element as defined in claim 1 wherein the Y section of the Y section fibers has legs of substantially equal length and of substantially equal shape and the angles between the legs of the Y are substantially equal.

3. A tobacco smoke filtering element as defined in claim 2 wherein the individual filaments have a surface lubricant comprising a pharmaceutical grade mineral oil.

4. A tobacco smoke filtering element comprising a substantially structurally unitary, elongated, rod-like mass of synthetic thermoplastic fibers and a wrapper encircling the mass, the mass comprising a segment of a continuous filament tow having 4 to 18 crimps per inch, said tow being a bundle of filaments spun from a plurality of holes in one spinnerette assembled and substantially parallelized with filaments spun substantially simultaneously from other spinnerettes and substantially every filament of the mass being substantially coextensive therewith, said tow having been treated to bring its filaments into substantially uniform cross-sectional distribution, the filaments of the mass being in general in substantial alignment longitudinally of the mass, a plurality of the filaments of the mass being fused to contiguous filaments at plasticized random points of contact, and at least a substantial portion of the filaments having a substantially uniform Y-shaped cross-section.

5. A tobacco smoke filter comprising an elongated mass of 5,000 to 100,000 dry-spun, thermoplastic fibers of 1.5 to 16 denier per fiber, said fibers being substantially oriented longitudinally of the mass, coextensive in length therewith, and coalesced to each other at random points,

said mass being a transversely-cut segment of a crimped tow of continuous filaments of a total denier of about 60,000 to about 250,000, and said filter being characterized particularly by the fact that the fibers have a substantially uniform Y-shaped cross-section.

6. A tobacco smoke filter comprising an elongated, cylindrical mass of 5,000 to 100,000 dry-spun thermoplastic fibers of 1.5 to 16 denier per fiber, said fibers being substantially oriented longitudinally of the mass,

10 substantially uniformly distributed across the cross-section of the mass, and coextensive in length with the mass, said mass being a transversely-cut segment of a crimped tow of continuous filaments of a total denier of about 60,000 to about 250,000, the mass comprising at least a substantial proportion of fibers having a uniform, 15 Y-shaped cross-section, the Y-section having legs of substantially equal length and of substantially equal shape, and the angles between adjacent legs of the Y preferably being substantially equal.

20 7. A tobacco smoke filter comprising an elongated, cylindrical mass of 5,000 to 100,000 cellulose acetate fibers of 1.5 to 16 denier per fiber, said fibers being substantially oriented longitudinally of the mass, substantially uniformly distributed across the cross-section of the mass,

25 coextensive in length with the mass, and coalesced to adjacent fibers at random points in plasticized portions of the fibers, said mass being a transversely-cut segment of a crimped tow of 4 to 18 crimps per inch of continuous filaments, the segment having a total denier of about 30 60,000 to about 250,000, the fibers having a uniform Y-shaped cross-section.

8. A tobacco smoke filtering element comprising a substantially structurally unitary, elongated, rod-like mass of 35 5,000 to 100,000 cellulose acetate filaments and a wrapper encircling the mass, the mass comprising a segment of a crimped tow of continuous filaments, said tow having 4 to 18 crimps per inch and being a bundle of filaments spun from a plurality of holes in one spinnerette 40 assembled with filaments spun from other spinnerettes and the filaments of said mass being substantially coextensive in length therewith, said tow having been treated to bring its filaments into substantially uniform cross-sectional distribution, the filaments of the mass being in general in substantial alignment longitudinally of the 45 mass, a plurality of the filaments of the mass being fused to adjacent filaments at plasticized random points of contact, and at least a substantial portion of the filaments having a substantially uniform, Y-shaped cross-section.

9. A tobacco smoke filtering element comprising a 50 substantially structurally unitary, elongated, rod-like mass of synthetic, thermoplastic, dry-spun filaments and a wrapper encircling the mass, the mass comprising a segment of a crimped tow of continuous filaments, said tow being a bundle of substantially parallelized filaments substantially simultaneously spun from a plurality of holes 55 in one spinnerette assembled with filaments spun from other spinnerettes and the filaments of said mass being substantially coextensive in length therewith, said tow having been treated to bring its filaments into substantially uniform cross-sectional distribution, the filaments of the mass being in general in substantial alignment longitudinally of the mass, a plurality of the filaments of the mass being fused to adjacent filaments at plasticized random points of contact, and at least a substantial portion 60 of the filaments having a substantially uniform, Y-shaped cross-section.

10. An article of manufacture comprising an intermediate product for use in the manufacture of fibrous cigarette filter tip elements of which the fibers are parallelized and coextensive, said intermediate product being a packaged, substantially untwisted, elongate, crimped, continuous filament tow of 5,000 to 100,000 filaments which in the aggregate are substantially parallel, the filaments being an unplasticized but plasticizable, dry-spun, 70 cellulose acetate having an acetyl content of about 75

38-41%, the filaments being of about 1.5 to about 16 denier per filament, the tow having about 4 to 18 crimps per inch and the total denier of the tow being within the range of about 60,000 to about 250,000, the tow having a low degree of lubrication provided by a small amount, of the order of about 0.5% by weight, of a non-toxic lubricant comprising a pharmaceutical grade mineral oil and at least a substantial portion of the filaments having a substantially uniform, Y-shaped cross-section, the crimp, the low order of lubrication, and the shape and character 10 of the Y-shaped filaments providing the tow with good blooming qualities and at least a substantial portion of the filaments having a substantially uniform, Y-shaped cross-section.

11. A packaged article of manufacture comprising an 15 intermediate product as defined in claim 10 wherein the Y section of the Y-shaped filaments of the tow has legs

5 of substantially equal shape and the angles between adjacent legs of the Y preferably are substantially equal.

**References Cited in the file of this patent**

**UNITED STATES PATENTS**

|           |          |               |
|-----------|----------|---------------|
| 1,480,463 | Petzel   | Jan. 8, 1924  |
| 1,773,969 | Dreyfus  | Aug. 26, 1930 |
| 1,944,378 | Thenoz   | Jan. 23, 1934 |
| 2,259,150 | Childs   | Oct. 14, 1941 |
| 2,476,582 | Browne   | July 19, 1949 |
| 2,483,406 | Francis  | Oct. 4, 1949  |
| 2,508,799 | Reis     | May 23, 1950  |
| 2,637,893 | Shaw     | May 12, 1953  |
| 2,688,380 | MacHenry | Sept. 7, 1954 |

**FOREIGN PATENTS**

|         |               |               |
|---------|---------------|---------------|
| 665,278 | Great Britain | Jan. 23, 1952 |
|---------|---------------|---------------|

U. S. DEPARTMENT OF COMMERCE  
PATENT OFFICE

**CERTIFICATE OF CORRECTION**

Patent No. 2,828,752      Wallace T. Jackson      April 1, 1958

It is hereby certified that error appears in the printed specification of the above numbered patent requiring correction and that the said Letters Patent should read as corrected below.

Column 1, line 69, strike out "only"; column 7, line 19, for "filaments 25" read --filaments 25Y--; column 9, line 32, for "among" read --amount--; line 59, for "sufficiently" read --sufficient--; column 10, line 22, for "two" read --tow--.

Signed and sealed this 24th day of June 1958.

(SEAL)

Attest:

KARL H. AXLINE

Attesting Officer

ROBERT C. WATSON  
Commissioner of Patents